

Nov. 28, 1967

D. A. ROSS

3,354,511

## TEXTILE CRIMPING

Filed Jan. 21, 1965

2 Sheets-Sheet 1



Nov. 28, 1967

D. A. ROSS

3,354,511

TEXTILE CRIMPING

Filed Jan. 21, 1965

2 Sheets-Sheet 2



*Fig. 6.*

1

3,354,511

## TEXTILE CRIMPING

Donald Alexander Ross, Sudbury, Mass., assignor to International Wool Development Company, Melbourne, Victoria, Australia, a proprietary limited  
Filed Jan. 21, 1965, Ser. No. 426,756  
11 Claims. (Cl. 19—66)

This invention relates to mechanical crimping of animal, vegetable, and synthetic textile materials in the form of spun yarn, multi-filament yarn, singles yarn, plied or folded yarn, slubbing, roving, sliver, top, tow, or sheets of fibers, such as card web.

A primary object of the invention is to provide a method for mechanically crimping such materials which can be reliably and economically practiced on relatively simple equipment which has both versatility with respect to the character of the crimping imparted to a single type of material, and a capacity, without complicated adjustment or interchange of parts, to accommodate a great variety of kinds and sizes of material.

A further object of the invention is to provide a method and apparatus for mechanically crimping such materials with less physical degradation, particularly in the case of wool, than is caused by present-day crimping techniques which apply such severe compressive forces to the fibers as to totally collapse them at spaced points and so weaken the fibers at the points of collapse as to cause tensile strength and elongation-at-break losses of up to 50% or even higher. Using the method and apparatus of this invention, crimping may be accomplished with little, if any, physical degradation.

Use of the invention permits, in addition to imparting crimp to normally uncrimped fibers for purposes of increasing resilience, compressibility, covering power, bulk or of increasing hand, upgrading crimped fibers of comparatively low natural crimp, such as the wool from certain breeds or having certain geographic origin.

In accordance with a preferred form of the invention, a textile strand material is continuously advanced along a pathway, in the course of which it is mechanically crimped by confining the continuously advancing strand against free lateral movement at two closely spaced lines of advance along its path of advance between which lines the strand runs freely suspended, and continuously changing the location of the first point of lateral confinement back and forth cross-wise of the general direction of strand advance while permitting the portion of the strand entering the second point of lateral confinement to substantially track the traversing motion at the first point as a result of the cross-force exerted by tension imposed upon the intervening suspended portion of the strand during its cross-motional egress from the first point of lateral confinement.

The cross-motion may be imparted to the strand at the second line of advance, in which case no cross-motion need, though it can also be, imparted to the strand at the first line of advance.

In both cases, the lateral location of the strand as it reaches the second line of advance moves back and forth along the transverse projection of the angularly advancing increment of yarn running between the two lines of advance.

Strand advance is caused by utilizing at the second line of advance opposed surfaces in the form of rollers or belts driven at a constant speed and forming a converging nip. The surfaces at the second line of advance define an elongated entrance slot leading, in the case of belts, into a flat laterally elongated confining passageway, the slot being of such width that the strand may enter the slot at various positions widthwise of the passageway and therefore traverse the slot laterally while con-

2

tinuously advancing into engagement between the constantly moving surfaces which grip the running strand against bodily transverse motion. Use of endless belts to form the confining passageway permits the belts to carry the strand gripped in the configuration it acquires upon entering the slot as a single layer along a planar pathway for such distance as may be required to perform such further treatment as is needed, or desirable, to set the configuration of the strand.

Preferably, the strand is gripped at the first line of advance also by a pair of surfaces moving in the direction of yarn advance, though in certain cases, it may suffice to confine it merely by running it through a trough, eye, or other laterally confining guide.

In the case of strand material, such as slivers having low tensile strength, both sets of moving surfaces are preferably driven with the first set operating usually at a higher surface speed than those at the second station but, in some cases of discontinuous fibrous strands at a less speed.

The above and other objects of the invention will be more clearly understood when taken in connection with a description of the structure and operation of typical apparatus designed to practice crimping methods of the invention, as illustrated in the accompanying drawings wherein:

FIG. 1 is a schematic view of essential operating parts of an apparatus performing a crimping operation in accordance with the principles of the invention;

FIG. 2 is a schematic plan view of the parts and operation shown in FIG. 1, showing certain parts in dotted line position;

FIG. 3 is a front end view, showing certain parts in cross-section, of a suitable apparatus for practicing crimping methods of the invention;

FIG. 4 is a vertical cross-sectional view taken along the line 4—4 of FIG. 3;

FIG. 5 is a schematic view, similar to that of FIG. 1, showing a modified form of operation;

FIG. 6 is a front end view, partly in cross-section, of a modified form of apparatus designed to practice the principles schematically illustrated in FIG. 5.

FIGS. 1 and 2 show a pair of juxtaposed gripping and feeding rolls 10 and 12 forming a nip which is horizontally aligned with a nip formed by a second pair of gripping rolls 14 and 16, one of which is a constant speed driving roll. The rolls 10, 12 are mounted for simultaneous bodily reciprocation along their axes. A pair of laterally spaced guide pins 18, which reciprocate with rolls 10 and 12, lead wool sliver, as an example, between the feed rolls 10 and 12 constituting a first station. As the sliver proceeds beyond the feed rolls 10 and 12, it is pulled between the rolls 14, 16 constituting a second station. Reciprocating motion of the feed rolls 10 and 12, as indicated in FIG. 1 and as illustrated by the movement of the feed roll 10 and guide pins 18 from their full-line positions in FIG. 2 to their dotted line positions in FIG. 2, causes the sliver to leave the rolls 10 and 12 at constantly changing lateral positions so that the increment of sliver suspended between the two sets of rolls runs angularly and therefore causes an angular entrance of the individual sliver fibers into the second set of rolls, tracking the path of the sliver's egress from the first set of rolls. The reversing of the angularity at the terminal of each reciprocation produces a bending of the fibers so that they merge from between the two rolls 14 and 16 with a crimped configuration, the character of which depends upon the particular settings of the variables, including the relationship between the speed of the reciprocation cycle and the rate of sliver advance, the pattern of reciprocation, the geometry of the spacing between and the relative speeds of the two sets of rolls, the pressure applied

in FIG. 1 and as illustrated by the movement of the feed roll 10 and guide pins 18 from their full-line positions in FIG. 2 to their dotted line positions in FIG. 2, causes the sliver to leave the rolls 10 and 12 at constantly changing lateral positions so that the increment of sliver suspended between the two sets of rolls runs angularly and therefore causes an angular entrance of the individual sliver fibers into the second set of rolls, tracking the path of the sliver's egress from the first set of rolls. The reversing of the angularity at the terminal of each reciprocation produces a bending of the fibers so that they merge from between the two rolls 14 and 16 with a crimped configuration, the character of which depends upon the particular settings of the variables, including the relationship between the speed of the reciprocation cycle and the rate of sliver advance, the pattern of reciprocation, the geometry of the spacing between and the relative speeds of the two sets of rolls, the pressure applied

between each pair of rolls, and the temperature of the rolls.

FIGS. 3 and 4 show the apparatus in more detail, adding, in particular, a confining passageway trailing the rolls 14 and 16 through which the crimped sliver may advance in a single layer while being further treated to increase the permanency of the set of the crimps imparted at the rolls.

Referring to FIG. 4, frame 20 of the machine supports two opposed flat endless belts 21 and 22 formed preferably of steam permeable fabric having low elongation characteristics and passing over front end rollers 23, 24 and 25, 26, respectively, and rear end rollers 27 and 28. The adjacent traverses of the belts 21 and 22 form an open-ended planar passageway having an entrance in the form of an elongated transverse slot 29. The passageway extends through a steam box 30 of conventional construction. Rolls 27 and 28 are driven as through a common chain drive 31 to drive belts 21 and 22.

At the front end of frame 20, a depending bar 40 and an upstanding bar 42 form a pair of parallel opposed horizontal laterally extending guide rails which are slideably engaged by bifurcated top and bottom ends of spaced side plates 44 and 45 of an intervening carriage 46. Side plates 44 and 45 are bolted together by tie rods 47 and 48.

An upper feed roll 50 and a lower feed roll 52 are mounted in suitable bearings for rotation between the side plates 44 and 45. In order to drive lower roll 52, its shaft extends through side plate 44 and frame 20 and assumes a square configuration for insertion into a square bore of a drive pulley 53 journaled in a bearing 54 fixed on frame 20. Such construction is well known as a means for driving feed roll 52 while the roll 52 reciprocates on carriage 46. Roll 50 is preferably spring-loaded (not shown) to insure that the rolls firmly grip strand material passing therebetween. Provision may be made for heating any or all of rolls 50, 52, 24 and 25 as by using hollow rolls through which heated water or steam may be circulated, or by inserting electrical heating units.

Reciprocation of carriage 46 relative to rail bars 40 and 42 is imparted in FIG. 3 by a crank 60 pivotally connected to a suitable extension 61 which is fixed on the outer side of side plate 45, though other reciprocating drives may be used depending upon what particular periodic motion is desired.

Side plates 44 and 45 also support forwardly extending ear plates 62 and 63 which suspend therebetween a vertically adjustable platform 64 carrying two upstanding laterally spaced guide pins 65 and 66, which correspond to the rods 18 shown in FIGS. 1 and 2, and may be mounted for lateral adjustment. The distance between feed rolls 50 and 52 and the vertical reaches of belts 21 and 22 may also be adjusted by moving rails 40 and 42 and the accompanying drive mechanism back and forth longitudinally on the frame 20.

FIG. 5 schematically illustrates a modification wherein the feed rolls 10 and 12, instead of reciprocating, have periodic motion by moving through an orbital path. One means for imparting such orbital motion is shown in FIG. 6 wherein upper and lower feed rolls 50 and 52, platform 64, and guide pins 65 and 66 are arranged as in FIGS. 3 and 4. However, carriage side plates 44a and 45a, instead of being engaged by opposed rails, are hung on a cross rod 70 whose ends are free to reciprocate vertically in opposed vertical slots 71 in frame 20. The bottoms of side plates 44a and 45a are adjustably fixed to a yoke 72 whose legs are pivoted to a pair of drive discs 73 and 74, driven in synchronism by a common drive belt 75 by motor 76 through gear box 77. Roll 52 is driven through a pulley 78 which, unlike pulley 53 in FIG. 4, is not attached to frame 20, but orbits with carriage 46a. Its drive belt 79 is sufficiently elastic to accommodate this orbital motion without interrupting the drive of feed roll 52.

Periodic orbital motion has certain advantages over

the reciprocating motion utilized in FIGS. 3 and 4. Apparatus-wise, it lessens vibration, and process-wise it tends more nearly to equalize the length of the increment of material suspended between the two sets of rolls throughout each cycle. In FIGS. 3 and 4, during reversals of the feed roll motion, slack may occur momentarily in the suspended increment of sliver which must pass through a condition of parallelism to the direction of belt advance with each reversal of the angularity of feed to the belt passageway. This momentary slack can be partly or wholly taken up by including the relative up and down motion provided by the orbital path. In addition, if desired, the feed rolls may move towards and away from the rolls 14 and 16 twice in each cycle so that at both extremities of their bodily transverse motion they are at their limit of motion towards rolls 14 and 16. Thus in the case of FIGS. 1 and 2, the back and forth motion of the feed rolls 10 and 12 will be along an arcuate path; while in the case of FIG. 5, the path of motion will be along the boundary of a saddle. Each of these motions tend to more equally control the strain on the increment of yarn suspended between the pairs of rolls by regulating its length throughout the cycle. These alternative paths of motion are indicated by the double-ended arrows in FIGS. 1, 2 and 5.

#### Example I

A card sliver of New Zealand Romney cross-bred wool of 46s quality number was gilled once to form a sliver of 5,500 tex. The material was fed at atmospheric conditions through the apparatus shown in FIGS. 3 and 4 with the feed rolls operating at a speed of 18 inches per minute and the receiving belts running at 16 inches per minute, the distance between the point of egress from the feed rolls and the point of entry into the belts being a distance of about  $\frac{3}{4}$  inches. The feed mechanism was reciprocated at 60 cycles per minute over a traverse of 3.25 inches.

The steam box was 25 inches in length so that the fibers were steamed for 1.6 minutes with steam entering the steam box at 7 p.s.i.

The resulting wool sliver contained several rows of crimps per inch.

Comparative tensile tests of the Romney cross-bred wool gave mean values of 13.0 g./tex breaking load and 32.0% elongation at break before crimping with losses of only 1.2% in breaking load and of only 5.8% in elongation at break after crimping. These results contrasted with losses of 56.8% in breaking load and 79.3% in elongation at break when the same wool was crimped in a commercial nylon stuffer box crimper.

Lowering the feed roll speed down as far as 14 inches per minute failed to change appreciably the appearance of the crimp and was regarded as desirable in imposing more tension on the suspended increment of the strand and hence greater stress conducive to more permanence in the crimp.

#### Example II

The procedure of Example I was followed except that the sliver was wet out with water prior to being fed to the apparatus.

#### Example III

The procedure of Example I was followed except that the sliver was additionally steamed prior to entering the feed rolls.

#### Example IV

The procedure of Example I was followed except that the sliver was additionally steamed between the feed rolls and the belt nip.

#### Example V

The procedure of Example I was followed except that the sliver was additionally steamed both before and after going through the feed rolls.

Examples II, III, IV and V produced results similar

to the product of Example I.

5  
*Example VI*

The procedure of Example I was followed except that the sliver was additionally first wet out with a 1% aqueous solution of sodium bisulphite at room temperature and then passed through squeeze rolls to remove excess water before being brought to the feed rolls. If the treated sliver is dried, it is desirable to add moisture (either by steaming or padding) before the setting operation. The bisulphite treatment assists in setting the crimp and merely exemplifies one of the conventional setting agents heretofore used for such purposes in connection with other mechanical crimping processes. Others are, for example, sodium thioglycollate, ethanolamine, and monoethanolamine sulfite.

*Example VII*

Utilizing the same apparatus settings set forth in Example I, a 6,000 tex sliver of 15 denier, 3.5 inches nylon polyamide was passed through the apparatus in accordance with the procedure of Example I. The resulting crimped sliver exhibited several rows of crimps per inch.

Similar results were secured with a 6,000 tex sliver of 3 denier, 4.5 inches orlon polyacrylic fiber, a 9,000 tex sliver of 4.5 denier, 4.5 inches Dacron polyester fiber and with a 7,800 tex sliver of linen flax vegetable fiber.

*Example VIII*

The drive to feed roll 52 was disconnected so that rolls 50 and 52 rotated freely. Wool sliver, woolen and worsted and synthetic yarn were successfully crimped.

Mono-filament yarns may also be crimped by either a single feed or in simultaneous multiple feed. Multiple feeds may also be used for other strand materials, depending upon the width of the apparatus. Strand material as used herein is not intended to exclude lengthwise components of strands contained in open weave woven or other fabrics where such components are sufficiently free to be flexed into crimped configuration.

In general, the cross motion may be in the range of 1 to 5 inches where the shortest suspended increment of material between feed rolls and belts will be of the order of  $\frac{1}{2}$  inch in length, the belt speed is 16 inches per minute, and the cross-motion cycle is varied between 30 and 240 cycles per minute, but could be higher, particularly for synthetics. As previously described, the feed roll speed may be in a ratio to the belt speed of less or more than 1:1. Increasing the ratio to as much as 3:2, however, lessens the crimp. Belt speeds up to 34 inches per minute also have been used successfully. In general, the shorter the distance between the roll pairs, the less the required traverse.

Referring to FIGS. 1, 2 and 5, it can be understood that the relative motions of the two sets of rolls can be imparted by periodic lateral motion of the second set of rolls 14 and 16, rather than of the first set, or by out-of-phase periodic lateral motion of both sets of rolls. Either of these modifications is, however, more complex where belts are used, as in FIG. 3.

What is claimed is:

1. The method of imparting artificial crimp to fibrous and filamentary textile strand material which comprises advancing said strand material while confining the strand as it advances against free lateral motion at two closely spaced lines of advance of the advancing strand, with the strand freely suspended between said lines, continuously moving the strand as it advances through at least one of said lines of advance back and forth transversely with respect to its general direction of advance to cause the lateral location of the strand as it reaches the second line of advance to move back and forth along the transverse projection of the angularly advancing increment of strand running between said two lines to continuously reversely flex the strand laterally at such a frequency as to produce closely connected crimps lengthwise along said strand material and carrying the crimped strand in crimped con-

## 6

figuration along a constant path beyond said second line of advance.

2. The method as claimed in claim 1, wherein the strand material is wool sliver.

5 3. The method as claimed in claim 1, wherein the strand material is wool sliver pre-wetted with an aqueous sodium bisulphite solution.

4. The method as claimed in claim 1, including gripping the strand against bodily transverse motion at the second line of advance.

5. The method as claimed in claim 1, wherein the strand is reversely flexed into single layer crimped configuration with the side edges of the layer continuously embracing a straight line running longitudinally medially of the layer.

10 6. The method of imparting artificial crimp to fibrous and filamentary textile strand material which comprises advancing said strand material while gripping the strand against free lateral motion at two separated, but closely spaced, lines of its advance, with the strand freely suspended between said lines, continuously moving the strand as it advances through at least one of said gripping stations back and forth transversely with respect to its general direction of advance to cause the lateral location of the strand as it reaches the second line of advance to move back and forth along the transverse projection of the angularly advancing increment of strand running between said two stations, to continuously reversely flex the strand at such a frequency as to produce closely connected crimps 15 lengthwise along said strand material and carrying the crimped strand in crimped configuration along a constant path beyond said second line of advance.

7. The method of imparting artificial crimp to fibrous and filamentary textile strand material which comprises advancing said strand material while gripping the strand against free lateral motion at two closely spaced stations of its advance, with the strand freely suspended between said lines, continuously moving the strand as it advances through the first of said stations back and forth trans-

35 versely with respect to its general direction of advance to cause the lateral location of the egress of the strand from the first gripping station to move back and forth and cause the strand to be received in the second gripping station at varying locations tracking the cross-motion of the strand at the first station with the increment of strand material 40 between said stations running in periodically reversing angular directions under tension at such a frequency as to continuously reversely flex the strand to produce closely connected crimps lengthwise along said strand material 45 and carrying the crimped strand in crimped configuration 50 along a constant path beyond said second line of advance.

8. Apparatus for crimping textile strand material comprising a pair of endless flat belts mounted in juxtaposed relation for unidirectional movement along close parallel 55 opposed traverses and forming a flat, laterally elongated passageway therebetween, said belts forming a converging nip defining a slot at the entrance to said passageway for gripping strand material fed into said nip at any location along said slot, a pair of opposed strand-gripping rolls

60 disposed in closed proximity to said nip for guiding strand material from said rolls directly into said nip and means for traversing said rolls back and forth in front of said nip at such frequency as to impose tension upon said strand material and cause it to advance from said rolls 65 into said nip with reversing angularity and means for driving at least one of said belts to move the strand through said passageway.

9. Apparatus for crimping textile strand material as claimed in claim 8 having means to drive at least one of 70 said rolls at a surface speed different from the surface speed of said belts.

10. Apparatus as claimed in claim 8, wherein the gripping nip between said rolls lies in the plane of said passageway in parallelism with said slot.

11. Apparatus for crimping textile strand material com-

prising a pair of endless flat belts mounted in juxtaposed relation for unidirectional movement along close parallel opposed traverses and forming a flat, laterally elongated passageway therebetween, said belts forming a converging nip defining a slot at the entrance to said passageway for gripping strand material fed into said nip at any location along said slot, means disposed in close proximity to said nip for guiding strand material into said nip and means for moving said guiding means in an orbital path in front of said nip to impose tension upon said strand material and cause it to advance into said nip in traversing relation back and forth along said slot and means for driving at

least one of said belts to move the strand through said passageway.

**References Cited:****UNITED STATES PATENTS**

|   |           |         |                |        |
|---|-----------|---------|----------------|--------|
| 5 | 2,184,390 | 12/1939 | Lovett         | 242-43 |
|   | 3,058,167 | 10/1962 | Rainard et al. | 28-72  |
|   | 3,083,437 | 4/1963  | Davis          | 19-160 |
|   | 3,112,054 | 11/1963 | Fleissner      | 28-72  |

10 MERVIN STEIN, *Primary Examiner.*

I. C. WADDEY, *Assistant Examiner.*